# EUROPEAN PATENT SPECIFICATION

(11) **EP 2 086 705 B1**
(45) Date of publication and mention of the grant of the patent: **17.08.2011**
(21) Application number: 07711456.9
(22) Date of filing: 07.02.2007
(51) Int. Cl.: B22D 13/06, F01D 5/00

(54) **METHOD FOR PRODUCTION OF TURBINE BLADES BY CENTRIFUGAL CASTING**
VERFAHREN ZUR HERSTELLUNG VON TURBINENSCHAUFELN DURCH SCHLEUDERGIESSEN
PROCÉDÉ DE PRODUCTION D'AUBES DE TURBINE PAR COULÉE PAR CENTRIFUGATION

(30) Priority: 23.10.2006 WO PCT/EP2006/010191
(43) Date of publication of application: 12.08.2009
(73) Proprietor: Renkel, Manfred, 96231 Bad Staffelstein (DE)
(72) Inventor: Renkel, Manfred, 96231 Bad Staffelstein (DE)
(74) Representative: Gassner, Wolfgang
(86) International application number: PCT/EP2007/001024
(87) International publication number: WO 2008/049465

(56) References cited:
- JP-A- 6 033 701
- JP-A- 55 081 052
- US-A- 5 284 620
- US-A- 5 671 533
- US-A1- 2004 060 685

## Description

The invention pertains to a method for production of turbine blades by centrifugal casting. The method in particular pertains to the production of turbine blades made of titanium or alloys containing large amounts of titanium, e. g. titanium aluminides.

Especially titanium aluminides are considered an optimum material in various areas of application because of their low density, relatively high-temperature, specific strength relative to nickel superalloys, and corrosion resistance. However, materials with a narrow range between solidus and liquidus temperature, like TiAl or pure titanium grade 2, are very difficult to shape, the only practical method for forming them is to cast them.

When casting such materials one is encountered with further problems live an unusual high amount of shrinkage of the intermetallic phase (γ-TiAl) during solidification resulting in the formation of shrinkholes, voids, pores, etc. in castings. This makes it usually necessary to reprocess the casting by expensive high-pressure compaction (HIP method).

Further, when casting such materials in molds having a complicated geometry, like shrouded tubine blades, the casting frequently shows damages shows damages like cracks, e. g. hot tears, or even torn off blade shrouds. These are strain induced damages corresponding to a rapid shrinkage during the solidification process.

An object of the present invention is it to avoid the disadvantages in the art. It is an aim of the present invention to provide a method allowing a production of castings having less pores, shrinkholes, voids and the like, thereby avoiding an expensive reprocessing by high-pressure compaction. A further aim of the present invention is to provide a method by which castings having a complicated geometry can be produced without strain induced damages.

US-A-5,950,706 describes a method for production of valves by centrifugal casting. A mold for forming the valves is arranged in a radial direction relative to an axis of the rotor. A rotational axis of the mold coincides with the radial direction.

US 5,671,533 describes the use of centrifugal casting in the manufacture of airfoils made from titanium alloys

This object is solved by the features of claim 1. Advantageous embodiments of the invention are described by the features of claims, 2 to 16.

In accordance with the present invention there is provided a method for production of a turbine blades by centrifugal casting, the turbine blade having a leading edge portion with a first thickness and a flowing-off edge portion with a second thickness being smaller than the first thickness, comprising then following steps:
a) providing a centrifugal casting device having a rotor being rotatable around an axis, and at least one crucible being accommodated in the rotor, the crucible having at least one outlet opening,
b) providing a mold having an extended cavity for forming the turbine blade,
c) arranging the mold at a radially outward position with respect to the crucible, so that an inlet opening of the mold is arrange vis-a-vis with an outlet opening of the crucible, and further arranging the mold so that a mold leading edge, which corresponds to the leading edge of the turbine blade, is directed in a direction against the rotational direction of the rotor,
d) rotating the rotor and thereby forcing a metal melt by means of centrifugal forces from the crucible into the mold,
e) exerting a pressure on the melt being forced into the mold until the temperature of the solidifying melt has reached a predetermined cooling-temperature, and
f) relieving the pressure when the temperature of the solidifying melt is smaller than said predetermined cooling-temperature.

In the sense of the present invention under a "crucible" there is in general understood a container which has sufficient heat resistance to take up a metallic melt without being damaged and without undergoing reactions with the metal melt. A "crucible" in the sense of the present invention may have any suitable shape. In particular it may have a cylindrical shape the bottom of which has a rounded concave shape. However, a "crucible" in the sense of the present invention may also be formed as a ring-like channel. Suitable materials for the production of a crucible are alumina, Y₂O₃, magnesia, silica glass, graphite and the like.

A turbine blade is in its cross section formed similar like a wing of an aircraft. The turbine blade has a leading edge portion with a first thickness and a flowing-off edge portion with a second thickness being smaller than the first thickness.

According to the invention it is provided that a mold leading edge which corresponds to the leading edge of the turbine blade is directed in a direction against the rotational direction of the rotor. Under the term "against the rotational direction of the rotor" it is understood that the mold leading edge is arranged either in coincidence with a radial plane of the rotor or is arranged at an angle of up to +/-90° with respect to the radial plane, said angle opening against the direction of rotation of the rotor. Under the "term radial" plane there is understood a plane which runs perpendicular to the rotational axis of the rotor.

By arranging the mold with its mold leading edge against the rotational direction of the rotor surprisingly the formation of pores and shrinkholes within the turbine blade, in particular within the leading edge portion thereof, can be avoided. It is assumed that when arranging the mold as proposed by the invention due to Coriolis-forces a higher pressure is exerted upon the melt in the leading edge portion than if the leading edge of the mold would be arranged in the rotational direction of the rotor.

According to an embodiment of the invention a connecting plane connecting the mold leading edge and the mold flowing-off edge is arranged with an angle of 2° to 45° relative to a radial plane of the rotor. Further, The leading edge can be arranged not only in parallel with a radial direction but also at a first angle α1 relative to the radial direction of the rotor. Preferably the first angle α1 opens in a direction against the direction of rotation of the rotor. That means that the mold may be arranged such that the leading edge is inclined in a direction against the rotational direction of the rotor. The first angle α1 may be up to 30°. By the aforementioned measures a further reduction of pores and shrinkholes in the casting can be achieved.

According to a further embodiment of the method the mold leading edge may be arranged in an axial plane at a second angle α2, of preferably up to 30°, relative to the radial direction of the rotor. Preferably the second angle α2 opens in a direction in which gravity acts. That means that the leading edge may be inclined with respect to the radial or horizontal plane at a first and/or second angle. Also this measure has the effect of reducing pores and shrinkholes.

The method according to the invention differs further from conventional methods in particular in that there is exerted a pressure on the melt after the mold has completely been filled.

The pressure may be exerted on the melt until the predetermined cooling-temperature is in a range of 1300°C to 800°C. The predetermined cooling-temperature depends on the used metal alloy. The predetermined cooling-temperature is advantageously selected to be lower than a brittle-ductile transition temperature of the used alloy. Under the term "brittle-ductile transition temperature" there is understood a temperature at which the bonds of an intermetallic phase change from metal bonds to atomic bonds. At temperatures above the brittle-ductile transition temperature intermetallic phases are bond by metal bonds. At such temperatures intermetallic phases are ductile. At a temperature below the brittle-ductile transition temperature intermetallic phases change their properties and become brittle. The predetermined cooling-temperature can be choosen to be for example 20°C to 200°C lower than the brittle-ductile transition temperature.

The amount of the pressure which is exerted on the melt after the mold is completely filled corresponds to the centrifugal force acting on the melt at the moment when the mold is completely filled times a factor of 1.0 to 5.0. The centrifugal force depends on the rotational speed of the rotor, the first radius at which the mold is distanced from the axis and the mass of the melt. Under the term "first radius" there is understood the distance between the axis and an inlet opening of the mold. According to the invention the pressure to be exerted on the melt is the centrifugal force at the precise moment of completely filling of the mold times a factor which is selected from a range of 1.0 to 5.0. From this relation one can calculate a suitable pressure to be exerted on the melt for molds being placed at a different first radius from the axis as well as for any mass of metal melt which is taken up in the mold. As can be seen from the above relation the pressure being exerted upon the melt after the mold is completely filled may be higher than during the time when the mold is being filled. According to an embodiment the pressure may be increased after the mold has been filled, preferably at a constant rate, for a predetermined period and afterwards there may be exerted a constant pressure on the melt. The predetermined period may be in the range of 1 to 25 seconds, preferably 5 to 20 seconds. The period of the constant pressure may be in range of 1 to 6 minutes, preferably of 4 to 6 minutes.

When reaching the predetermined cooling-temperature the pressure is relieved so that in maximum the atmospheric pressure is acting upon the melt.

By the proposed exerting of a pressure on the solidifying melt being hotter than the predetermined cooling-temperature a formation of pores, voids, shrinkholes and the like in the castings can be significantly reduced. It is in particular not necessary to reprocess the casting by high-pressure compaction. A particular advantage is that a formation of strain induced damages can be avoided even when producing castings with a complicated geometry, like shrouded turbine blades and vane clusters.

According to an advantageous embodiment the pressure exerted upon the melt is a constant or increasing pressure. In order to create the required pressure the rotor may be rotated with the same or an increasing speed during step lit. e).

According to a further embodiment of the invention the melt is heated up to a temperature which is 50°C to 150°C higher than the melting temperature of the metal. By this measure the heat energy of the melt is increased. When using such a superheated melt in particular an undesirable formation of cold runs in molds for castings having thick wall sections, i. e. sections with a thickness in the range of 0.5 mm, can be avoided.

According to a further advantageous feature the mold is preheated before step lit. c). The temperature of said preheating may be in the range of 50°C to 1100°C, preferably in the range of 850°C to 1100°C. Such a preheating temperature is in particular useful when producing turbine blades. For example for the production of turbo charger wheels it has been proofed to be advantageous to use a temperature for said preheating in the range of 50°C to 250°C. - It has to be understood that the preheating temperature of the mold depends from the geometry of the casting and has to be determined for each geometry.

The preheating of the mold can take place for example in a furnace from which the mold is transferred into the rotor before a centrifugal casting takes place. However, it is also possible to preheat the mold by suitable heating device being provided at the centrifugal casting device, in particular at the rotor. By preheating the mold an undesirable quenching of the melt being forced into the mold can be avoided. Surface quality of the casting can be improved. By preheating the mold in particular an undesirable reaction of the melt with the mold material can be counteracted.

According to a further advantageous feature the predetermined cooling-temperature is in a range of 1050°C to 800°C. Predetermined cooling-temperatures selected from this range are usually lower than the brittle-ductile transition temperature of titanium aluminides. When choosing a cooling-temperature from the proposed range and exerting a pressure upon the melt until the choosen predetermined cooling-temperature is reached castings made of titanium aluminides can be produced with an excellent quality.

The pressure can be exerted upon the melt in different manners. According to a simple embodiment the pressure is exerted upon the melt by rotating the rotor. In this case the pressure is created by centrifugal forces acting upon the melt. However, it is also possible to exert the pressure upon melt for example by pressurised gas. In this case as gas there may be used preferably an inert gas like Argon or the like.

According to a further embodiment of the invention during steps lit. d) and lit. e) the melt is under vacuum or shield gas. In particular the use of vacuum is advantageous as therewith a formation of gas-filled pores and an oxidation of the metal, in particular of titan aluminides, can be avoided. It has been proven appropriate to use a vacuum of 10⁻¹ to 10⁻² bar in order to avoid the formation of in particular gas-filled pores.

According to a further embodiment the solidifying melt is cooled down after step lit. e) to room temperature at a cooling-rate of 50°C to 150°C per hour. Such a cooling-rate can be realised by the use of molds having suitable thermal isolation properties. Molds without suitable thermal isolation properties may be placed in a furnace which is preheated upon a temperature which is in the range of the predetermined cooling-temperature. After transferring the mold into the furnace it may be cooled down by controlling the heating elements of the furnace so that the aforementioned cooling-rate is realised within the furnace. The proposed controlled cooling down of the mold also counteracts the formation of hot tears in the casting.

The proposed method is in particular well suited for producing castings from a metal melt consisting of a titanium alloy. The titanium alloy advantageously comprises Ti and Al as main constituents. A suitable composition (in at.%) of a γ-TiAl based alloy may be summarised as follows: $T ⁢ {i}_{45 - 52 ⁢ a ⁢ t . %} ⁢ A ⁢ {l}_{45 - 48 ⁢ a ⁢ t . %} ⁢ X ⁢ {1}_{1 - 3 ⁢ a ⁢ t . %} ⁢ X ⁢ {2}_{2 - 4 ⁢ a ⁢ t . %} ⁢ X ⁢ {3}_{1 ⁢ a ⁢ t ⁢ . %} ,$
where $X ⁢ 1 = C ⁢ r , M ⁢ n , V$ $X ⁢ 2 = N ⁢ b , T ⁢ a , W , M ⁢ o$ $X ⁢ 3 = S ⁢ i , B , C .$

For example, the titanium alloy may contain 30 to 45 wt.% Al, 1,5 to 6 wt.% Nb and as balance Ti as well as unavoidable impurities. The titanium alloy may further contain one or more of the further constituents: 0,5 to 3,0 wt.% Mn, 0,1 to 0,5 wt.% B, 1,5 to 3,5 wt.% Cr. Further, the titanium alloy may contain O in an amount of 0 to 1000 ppm, C in an amount of 0 to 1000 ppm, preferably 800 to 1200 ppm, Ni in an amount of 100 to 1000 ppm and N in an amount of 0 to 1000 ppm.

According to an embodiment of the invention the crucible is accommodated in the rotor at a second radial distance from the axis, the second radial distance being smaller than the first radial distance. The second radial distance may be calculated from an outlet opening of the crucible to the axis. Usually, the second radial distance is larger than a diameter of the crucible. If the crucible and the associated mold are both accommodated eccentrically with respect to the axis of the rotor it is possible to create higher centrifugal forces acting upon the melt at comparable rotating speeds. Thereby the mold can rapidly be filled and the formation of cold runs can be avoided. This further improves the quality of the casting in that less pores, voids or shrinkholes are created.

It is possible to create the melt in the crucible while the rotor is standing, i. e. while the rotor is not rotating. In this case the melt can be created by inductively heating an ingot within the crucible. It is also possible to heat the ingot or to support the heating of the ingot by microwaves. By the proposed heating methods an ingot can be melt within several minutes.

Alternatively, the metal melt may also be poured into the crucible. This allows a production of larger quantities of metal melt. If in the rotor there is accommodated a multitude of molds, a multitude of castings can be produced simultaneously.

According to a further embodiment the melt may be poured into the crucible while the rotor is rotating. By this measure the melt being poured into the crucible can be accelerated rapidly and can be forced with a high speed into the mold. Consequently, the mold is filled with the melt being at a relatively high temperature which in turn guaranties a certain mobility of the melt and therefore the pressure being exerted upon the melt during step lit. d) can effectively be used to cold runs and to reduce pores.

It has been proven appropriate that the crucible has the form of a ring-shaped channel being centrally accommodated in the rotor, the outer circumference of which having a second radial distance from the axis, the second distance being smaller than the first radial distance. According to this feature the melt is poured into a ring-shaped channel at a radial distance with respect to the axis. Consequently, the centrifugal force acting upon the melt and therefore the velocity by which the melt is transferred into the mold can be increased by this measure.

With respect to further embodiments of the alternative method reference is made to the above transcription of the embodiments regarding the method. The features described there can be also embodiments of the alternative method.

Embodiments of the invention are now described in detail with reference to the accompanied figures:
- Fig. 1: shows a sectional drawing of a first device,
- Fig. 2: shows a sectional drawing of a second device and
- Fig.3a: shows a first plot of the rotational speed of a ro- tor over the time,
- Fig. 3b: shows a second plot of the rotational speed of a rotor over the time,
- Fig. 4: shows a sectional drawing through an arm of the ro- tor of Fig. 1,
- Fig. 5: shows a sectional drawing according to the section line B-B in Fig. 4,
- Fig. 6: shows another sectional drawing according to Fig. 5,
- Fig. 7: shows another sectional drawing according to Fig. 5,
- Fig. 8: shows a sectional drawing through an embodiment of an arm of the rotor of Fig. 1, and
- Fig. 9: shows a sectional drawing through a further embodi- ment of an arm of the rotor of Fig. 1.

Fig. 1 shows a rotor 1 which is rotatable around an axis A. The rotor 1 comprises two hollow tube-like arms 2. At the outer end of each arm 2 there is realisably mounted, preferably in a gas-tight manner, a piston 3. In the piston 3 there is accommodated a mold 4 having a funnel-like inlet opening 5 which is directed to the axis A.

Nearby the outer end of each arm 2 there is provided a first crucible 6 made of a heat resistant material, e. g. silica glass or the like. The first crucible 6 is mounted at a bottom of the arm 2, preferably in a gas-tight manner.

The first crucible 6 is surrounded by an induction-coil 7 which can be moved in an essentially vertical direction. In an lower position (not shown here) of the induction-coil 7 it does not surround the first crucible 6 so that the first crucible 6 can be rotated with the rotor 1 around the axis A. Within the first crucible 6 there is accommodated a second crucible 8 having a outlet opening 9 which is placed opposite to the inlet opening 5 of the mold 4.

The second crucible 8 is made of a heat-resistant material, e.g. alumina, Y₂O₃, graphite or the like. According to a preferred embodiment of the invention the second crucible 8 is made of alumina, magnesia or the like. There may be provided a third crucible (not shown here) made of graphite which may be placed within the second crucible 8. By the use of the third crucible an inductive melting of an ingot taken up therein can be accelerated.

Opposite to a bottom of the second crucible 8 there is provided a window 10 through which by means of a camera 11 the melting of the ingot may be observed.

A hollow shaft 12 extending vertically from the rotor 1 may be driven by an electric motor (not shown here).

In an embodiment of the invention there is provided a vacuum source, e.g. a vacuum pump or the like, which is connected by means of a conventional sealing with the hollow shaft 12 to create within the rotor 1, which is designed in this case in a gas-tight manner, a vacuum.

In a second embodiment of the invention the rotor 1 may have breakthroughs 13. The rotor 1 may be surrounded by a gas-tight housing 14. The vacuum source may be connected to the gas-tight housing 14 to create therein and thereby also within the rotor 1 a vacuum.

In another embodiment of the invention there is provided instead of a vacuum source a source of a shield gas, e.g. Ar or the like, by which the hollow structure surrounded by the rotor 1 mary be flooded during the centrifugal casting process.

As can be seen from Fig. 1 the mold is accommodated within the rotor 1 at a first radial distance r1 and the second crucible 8 taking up a melt 15 is accommodated within the arm 2 at a second radial distance r2. Under the first radial distance there is understood a distance between then inlet opening 5 and the axis A; under the second radial distance there is understood the distance between the outlet opening 5 and the axis A. As can be seen from fig. 1 the first radial distance is larger than the second radial distance. Further, the second crucible has a cylindrical shape and the second radius is larger than the diameter of the crucible, i. e. the second crucible 8 is located eccentrically with respect to the axis A within the rotor 1.

It has to be understood that the rotor 1 may comprise more than two arms 2, e. g. 4, 6, 8 or more arms. The rotor 1 may also be disk-shaped.

According to a further embodiment within the rotor 1 there may also be accommodated a first and a second crucible which are formed like ring-channels. These ring like channels again may be made for example of a heat-resistant ceramic like silica-glass, alumina, graphite and the like. One or more ingots taken up in the second crucible, which is formed as a ring-channel, may be again heated by an induction-coil, which surrounds an inner and an outer diameter of the first crucible, which is as well formed like a ring-channel and which accommodates the second ring-channel like crucible.

The second ring-channel like crucible may have several outlet openings. Vis-à-vis each outlet opening there is accommodated in a radial direction a corresponding mold with their inlet opening.

Fig. 2 shows a second device in the rotor 1 of which there is centrically accommodated a fourth crucible 16, which may be made of alumina, Y₂O₃ or the like. Vis-à-vis second openings 9 of the fourth crucible 16 there are provided molds 2 with their inlet openings 5 being located vis-à-vis the outlet openings 9. The inlet openings 5 are arranged again in a first radial distance r1 from the axis A.

The fourth crucible 16 is arranged centrically with resepct to the axis A. A lid 17 having a centrically arranged opening 18 covers the fourth crucible 16. A fifth crucible 19 may be connected via a tube 19a with the opening 18 so that a melt can be poured from the fifth crucible 19 through the opening 18 into the fourth crucible 16.

By using the first device a precision casting may be produced as follows:
A titanium aluminide ingot is placed in the second crucible 8. The respective titanium aluminide alloy may have e. g. one of the following compositions:
   a) 31 wt.% Al, 5,wit.% Nb, 1.5 wt.% Mn, 0.3 wt.% B and as balance Ti as well as unavoidable impurities;
   b) 43 wt.% A1, 2 wt.% Nb and as balance Ti as well as unavoidable impurities;
   c) 33 wt.% A1, 5 wt.% Nb, 2,5 wt.% Cr and as balance Ti as well as unavoidable impurities.

A mold which may be made of a ceramic being lined at there interior contact surface with Y₂O₃ is preheated in a furnace up to a temperature of around 1000°C. Suitable materials for the production of a mold are for example disclosed in the WO 2005/039803 A2.

The mold 4 being preheated to a temperature of around 1000°C is mounted at the arm 2 and then covered with the piston 3 which is mounted in a gas-tight manner at the arm 2. In dependency on the number of arms 2 provided at the rotor 1 a multitude of molds 4 can be mounted at the rotor 1.

The ingot is then melt by inducing currents with the induction-coil 7. When the melt has reached a temperature in the range of 1400°C to 1700°C, preferably in the range of 1450°C to 1650°C, the rotor 1 is accelerated within 0.5 to 2.0 seconds, preferably within less than 1.5 seconds, upon rotational speed of 110 to 260 rpm, preferably with 100 to 160 rpm. The second radius r2 is in this case chosen to be 300 to 400 mm, preferably around 350 mm. The melt is forced by centrifugal forces from the second crucible 8 into the mold 4.

Afterwards the mold 4 has been filled with melt the rotor 1 is furtheron rotated at a rotational speed of 110 to 260 rpm, preferably of at least 160 rpm, for at least 60 seconds, preferably for 120 to 300 seconds. During the further rotation of the rotor 1 the rotational speed may be increased at a constant rate, e.g. from initial rotational speed selected from a range of 110 to 160 rpm to a rotational speed selected from a range of 180 to 260 rpm when the solidifying melt in the mold 4 has reached predetermined cooling-temperature in the range of 1300°C to 1100°C.

The temperature of the solidifying melt in the mold 4 may be determined by conventional temperature measuring techniques using for example a thermocouple. The temperature values measured therewith may be corrected in accordance with a suitable algorithm in a conventional manner.

When the rotation of the rotor 1 has been stopped the mold 4 is demounted from the arm 2 and then placed in the furnace which is preheated on a temperature of around 1000°C. The mold 4 is then cooled down within the furnace with a rate of 50°C to 100°C per hour.

According to an embodiment of the aforementioned method the rotor 1 may be evacuated before melting the ingot within the second crucible 8. The vacuum within the rotor 1 may be in the range of 10⁻¹ to 10⁻² bar. Alternatively the rotor 1 may be flooded with shield gas, for example Ar before melting the ingot.

By use of the second device precision castings by centrifugal casting can be produced as follows:

Molds 4 are preheated in a similar manner as described above in a furnace up to a temperature of 1000°C and then placed in suitable holding devices provided within the rotor 1.

The rotor 1 is accelerated upon a rotational speed in the range of 110 to 260 rpm. As soon as the melt has reached a predetermined temperature in the range of 1450°C to 1650°C the melt taken up in the fifth crucible 19 is poured into the fourth crucible 16. The melt is than forced through the outlet openings 9 provided at the fourth crucible 16 in the molds 4 which are located vis-A-vis.

Afterwards, the rotor 1 is furtheron rotated as described above. After stopping the rotation the molds 4 are demounted from the rotor 1 and cooled down as described above.

Figs. 3a and 3b show plots of the rotational speed of the rotor above the time. In Fig. 3a the acceleration of the rotor during the first 12 seconds from the beginning of the rotation is showed. Fig. 3b shows a rotational speed of the rotor from the beginning of the rotation until the rotation is stopped.

When using the first device an ingot is melt within the second crucible 8. As soon as predetermined temperature of the melt has been reached the rotor 1 is accelerated within less then one second up to a rotational speed of around 140 rpm. Observations have shown that the melt is completely forced into the mold one second after starting the rotation of the rotor 1. As can be seen from Fig. 3a it is preferred to increase the rotational speed of the rotor 1 after the first second from around 140 rpm with a constant rate of 200 to 280 rpm², preferably with a rate of 240 rpm², so that around 14 seconds after the beginning of the rotation a rotational speed of around 220 to 240 rpm has been reached. When reaching the predetermined maximum rotational speed in the range of 200 to 250 rpm the rotor is furtheron rotated at a constant rotational speed. As can be seen from Fig. 3b this rotational speed may be in the range of 220 to 240 rpm, in particular around 225 rpm. Around 220 to 240 seconds after the beginning of the rotation of the rotor 1 the rotation is stopped.

When using the second device shown in Fig. 2 the melt is poured from the fifth crucible 19 into the fourth crucible 16 for example around 0:5 to 1.0 seconds after the rotation of the rotor 1 has been started, e. g. at a moment when the rotor rotates with a speed of around 140 rpm. Then the rotational speed the rotor 1 may be increased as shown in Fig. 3a at a constant rate until the rotor 1 has reached a rotational speed in the range of 200 to 240 rpm. Then the rotor 1 may be rotated at a constant speed in the range of 200 to 250 rpm for around two to four minutes.

By the proposed exerting of a centrifugal force on the solidifying melt in particular the formation of hot tears can be successfully be avoided. In the production of castings made from titan aluminides it has been proven to be advantageous to stop the exerting of the centrifugal force after the solidifying melt has reached a temperature which is lower than the brittle-ductile transition temperature of the material. Further, it is advantageous to increase the centrifugal force after the mold has completely being filled at the time when the melt is hot and mobile.

Figs. 4 to 9 show in more detail the arrangement of the mold 4, in particular the cavity 20 thereof, with respect to a radial plane P and/or a horizontal plane HP of the rotor 1.

Fig. 4 shows a sectional drawing through an arm 2 of a rotor 1 like in Fig. 1. The cavity 20 of the mold 4 is extending in a radial direction. A mold leading edge 21 is arranged relative to the rotational direction R of the rotor 1 behind a axial plane P which includes the axis A and runs essentially in parallel to the radially extending side faces of the arm 2 or the piston 3. A mold flowing-off edge 22 is arranged at the opposite side of this axial plane P.

Fig. 5 shows a schematic cross-section along the section line B-B in Fig. 4. As can be seen therefrom the mold leading edge 21 is situated in the vicinity of a portion of the mold 4 having a first mold thickness T1 which corresponds to a first thickness of a turbine blade manufactured by use of such a mold 4. The mold flowing-off edge 2 is situated in the vicinity of a portion of the mold 4 having second mold thickness T2 which corresponds to a second thickness of a turbine blade manufactured by use of this mold 4. The axial plane P devides the cavity 20 into two parts, a first part P1 being situated in the rotational direction R and a second part P2 being arranged against the rotational direction R. According to the present invention the cavity 20 is arranged always such that the mold leading edge 21 lies in the second part P2, i.e. is arranged against the rotational direction R of the rotor 1. A connecting plane CP connecting the mold leading edge 21 and the mold flowing-off edge 22 forms a tilting angle γ with the horizontal plane HP.

Figs. 6 and 7 show for clarification that in this view also other arrangements of the mold leading edge 21 are possible. Also in the embodiments shown in Fig. 7 and 8 the mold leading edge 21 lies in the second part P2. According to a preferred feature of the invention the tilting angle γ is up to +/- 30° with respect to the radial or horizontal plane HP.

Figs. 8 and 9 show further embodiments of the invention. As can be seen from Fig. 8 the mold 4 can be arranged in the horizontal plane such that the mold leading edge 21 is inclined with respect to the axial plane P or the radial direction of the arm 2 or the piston 3, respectively, at a first angle α1. The first angle α1 opens in a direction against the rotational direction R of the rotor 1, i. e. the cavity 20 is inclined against the rotational direction R.

As can be seen from Fig. 9 it is also possible to arrange the mold 4 within the arm 2 or the piston 3, respectively, such that the mold leading edge 21 is inclined with respect to a horizontal plane HP at a second angle α2. The second angle α2 may open in a direction of gravity, as shown in Fig. 9. However, it is also possible that the second angle α2 opens in the opposite direction, i. e. against the direction of gravity.

It has to be noted that the embodiments shown in Figs. 8 and 9 can be combined, i. e. the mold leading edge 21 may be inclined at a first angle α1 with respect to the axial plane P as well as a second angle α2 with respect to the horizontal plane HP. The first α1 and/or second angle α2 may be preferably up to 30°.

In the embodiments shown in Figs. 8 and 9 the mold 4 is taken up in the arm 2 such that the mold leading edge 21 is inclined with respect to the axial plane P and/or horizontal plane HP. Therefore, the axial plane P and/or horizontal plane HP just partly traverses the mold cavity 20. However, also in the embodiments shown in Figs. 8 and 9 the mold 4 may be arranged such that the mold leading edge 21 is arranged in a direction against the rotational direction R of the rotor 1.

By the proposed arrangement of a mold leading edge 21 with respect to the axial plane P and/or horizontal plane HP there can be manufactured a turbine blade with a strongly improved internal structure, i. e. the formation of pores and shrinkholes can be reduced remarkably. It is assumed that this effect is caused by Coriolis-forces which act upon the melt being cast into the cavity 20. According to the present invention the mold 4 is arranged such that the Coriolis-forces act with a high efficiency upon the first portion of the mold 4 which has a high thickness. By the Coriolis-forces a high additional pressure is created by which the formation of pores and shrinkholes in this thick portion is remarkably reduced.

## Claims

1. A method for production of a turbine blade by centrifugal casting, the turbine blade having a leading edge portion with a first thickness and a flowing-off edge portion with a second thickness being smaller than the first thickness, comprising the following steps:
a) providing a centrifugal casting device having a rotor (1) being rotatable around an axis (A), and at least one crucible (8) being accommodated in the rotor (1), the crucible having at Least one outlet opening,
b) providing a mold (4) having an extended cavity (20) for forming the turbine blade,
c) arranging the mold (4) at a radially outward position with respect to the crucible (8), so that an inlet opening (5) of the mold (4) is arranged vis-a-vis with an outlet opening (9) of the crucible (8), and further arranging the mold (4) so that a mold leading edge (21), which corresponds to the leading edge of the turbine blade, is directed in a direction against the rotational direction of the rotor (1),
d) rotating the rotor (1) and thereby forcing a metal melt (15) by means of centrifugal forces from the crucible (8) into the mold (4),
e) exerting a pressure on the melt (15) being forced into the mold (4) until the temperature of the solidifying melt (15) has reached a predetermined cooling-temperature, and
f) relieving the pressure when the temperature of the solidifying melt (15) is smaller than said predetermined cooLing-temperature.

2. The method of one of the preceding claims, wherein the mold leading edge (21) is arranged in a radial plane (HP) at a first angle (α1), of preferably up to 30°, relative to the radial direction of the rotor (1).

3. The method of one of the preceding claims, wherein the first angle (α1) opens in a direction against the direction (R) of rotation of the rotor (1).

4. The method of one of the preceding claims, wherein the mold leading edge (21) is arranged in an axial plane (P) at an second angle (α2), of preferably up to 30°, relative to the radial direction of the rotor (1).

5. The method of one of the preceding claims, wherein the predetermined cooling temperature is in a range of 1300° to 800°C.

6. The method of one of the preceding claims, wherein the pressure corresponds to the centrifugal force acting on the melt (15) at the moment when the mold completely filled times a factor of 1.0 to 5.0

7. The method of one of the preceding claims, wherein the pressure is exerted upon the melt (15) for to 6 minutes after the predetermined cooling-temperature has been reached.

8. The method of one of the preceding claims, wherein the pressure exerted upon the melt (15) is a constant or an increasing pressure.

9. The method of one of the preceding claims, wherein the rotor (1) is rotated with the same or an increasing speed during step lit. e).

10. The method of one of the preceding claims, wherein the predetermined cooling-temperature is in a range of 1050°C to 800°C.

11. The method of one of the preceding claims, wherein the pressure is exerted upon the melt (15) by rotating the rotor (1).

12. The method of one of the preceding claim, wherein during steps lit. d) and lit. e) the melt (15) is under vacuum or shield gas.

13. The method of one of the preceding claims, wherein the solidifying melt (15) is cooled down to room temperature after step lit. e) at a cooling-rate of 50°C to 150° per hour.

14. The method of one of the preceding claims, wherein the metal melt (15) consists of a titanium alloy.

15. The method of one of the preceding claims, wherein the titanium alloy comprises Ti and Al as main constituents.

16. The method of the proceding claims, wherein the titanium alloy is a γ-TiAl based alloy of the following composition:
$T ⁢ {i}_{45 - 52 ⁢ a ⁢ t . %} ⁢ A ⁢ {l}_{45 - 48 ⁢ a ⁢ t . %} ⁢ X ⁢ {1}_{1 - 3 ⁢ a ⁢ t . %} ⁢ X ⁢ {2}_{2 - 4 ⁢ a ⁢ t . %} ⁢ X ⁢ {3}_{1 ⁢ a ⁢ t ⁢ . %} ,$
where $X ⁢ 1 = C ⁢ r , M ⁢ n , V$ $X ⁢ 2 = N ⁢ b , T ⁢ a , W , M ⁢ o$ $X ⁢ 3 = S ⁢ i , B , C .$

## Patentansprüche

1. Verfahren zur Herstellung einer Turbinenschaufel durch Schleuderguss, wobei die Turbinenschaufel einen Anströmkantenabschnitt mit einer ersten Dicke und einen Abströmkantenabschnitt mit einer zweiten Dicke aufweist, welche kleiner ist als die erste Dicke, umfassend die folgenden Schritte:
a) Vorsehen einer Schleudergussvorrichtung mit einem Rotor (1), welcher um eine Achse (A) drehbar ist, und zumindest einem Tiegel (8), welcher im Rotor (1) aufgenommen ist, wobei der Tiegel zumindest eine Auslassöffnung aufweist,
b) Vorsehen einer Gussform (4) mit einem sich erstreckenden Hohlraum (20) zum Formen der Turbinenschaufel,
c) Anordnen der Gussform (4) an einer radial äußeren Position bezüglich des Tiegels (8), so dass eine Einlassöffnung (5) der Gussform (4) gegenüber einer Auslassöffnung (9) des Tiegels (8) angeordnet ist, und weiterhin Anordnen der Gussform (4), so dass eine Anströmkante (21) der Gussform, welche der Anströmkante der Turbinenschaufel entspricht, in eine Richtung entgegen dem Drehsinn des Rotors (1) gerichtet ist,
d) Drehen des Rotors (1) und **dadurch** Zwingen einer Metallschmelze (15) mittels Zentrifugalkräften vom Tiegel (8) in die Gussform (4),
e) Ausüben eines Drucks auf die Schmelze (15), welche in die Gussform (4) getrieben wird, bis die Temperatur der sich verfestigenden Schmelze (15) eine vorbestimmte Abkühltemperatur erreicht hat, und
f) verringern des Drucks, wenn die Temperatur der sich verfestigenden Schmelze (15) kleiner ist als die vorbestimmte Abkühltemperatur.

2. Verfahren nach einem der vorhergehenden Ansprüche, wobei die Anströmkante (21) der Gussform in einer radialen Ebene (HP) in einem ersten Winkel (α1), von vorzugsweise bis zu 30°, relativ zur radialen Richtung des Rotors (1) angeordnet ist.

3. Verfahren nach einem der vorhergehenden Ansprüche, wobei der erste Winkel (α1) sich in eine Richtung entgegen dem Drehsinn (R) des Rotors (1) öffnet.

4. Verfahren nach einem der vorhergehenden Ansprüche, wobei die Anströmkante (21) der Gussform in einer axialen Ebene (P) in einem zweiten Winkel (α2), von vorzugsweise bis zum 30°, relativ zur radialen Richtung des Rotors (1) angeordnet ist.

5. Verfahren nach einem der vorhergehenden Ansprüche, wobei die vorbestimmte Abkühltemperatur in einem Bereich von 1300° bis 800°C liegt.

6. Verfahren nach einem der vorhergehenden Ansprüche, wobei der Druck zu einer auf die Schmelze (15) wirkenden Zentrifugalkraft zu dem Zeitpunkt korrespondiert, wenn die Gussform komplett gefüllt ist, multipliziert mit einem Faktor von 1,0 bis 5,0.

7. Verfahren nach einem der vorhergehenden Ansprüche, wobei der Druck auf die Schmelze (15) für 1 bis 6 Minuten ausgeübt wird, nachdem die vorbestimmte Abkühltemperatur erreicht worden ist.

8. Verfahren nach einem der vorhergehenden Ansprüche, wobei der auf die Schmelze (15) ausgeübte Druck ein konstanter oder ein steigender Druck ist.

9. Verfahren nach einem der vorhergehenden Ansprüche, wobei der Rotor (1) mit der gleichen oder einer steigenden Geschwindigkeit während des Schritts lit. e) gedreht wird.

10. Verfahren nach einem der vorhergehenden Ansprüche, wobei die vorbestimmte Abkühltemperatur in einem Bereich von 1050°C bis 800°C liegt.

11. Verfahren nach einem der vorhergehenden Ansprüche, wobei der Druck auf die Schmelze (15) durch Drehen des Rotors (1) ausgeübt wird.

12. Verfahren nach einem der vorhergehenden Ansprüche, wobei die Schmelze (15) während der Schritte lit. d) und lit. e) unter Vakuum oder Schutzgas ist.

13. Verfahren nach einem der vorhergehenden Ansprüche, wobei die sich verfestigende Schmelze (15) nach Schritt lit. e) bei einer Abkühlrate von 50°C bis 150°C pro Stunde auf Raumtemperatur abgekühlt wird.

14. Verfahren nach einem der vorhergehenden Ansprüche, wobei die Metallschmelze (15) aus einer Titanlegierung besteht.

15. Verfahren nach einem der vorhergehenden Ansprüche, wobei die Titanlegierung Ti und Al als Hauptbestandteile umfasst.

16. Verfahren nach einem der vorhergehenden Ansprüche, wobei die Titanlegierung eine Legierung auf der Grundlage von γ-TiAl mit der folgenden Zusammensetzung ist:
$T ⁢ {i}_{45 - 52 ⁢ a ⁢ t . %} ⁢ A ⁢ {l}_{45 - 48 ⁢ a ⁢ t . %} ⁢ X ⁢ {1}_{1 - 3 ⁢ a ⁢ t . %} ⁢ X ⁢ {2}_{2 - 4 ⁢ a ⁢ t . %} ⁢ X ⁢ {3}_{1 ⁢ a ⁢ t ⁢ . %} ,$
wobei $X ⁢ 1 = C ⁢ r , M ⁢ n , V$ $X ⁢ 2 = N ⁢ b , T ⁢ a , W , M ⁢ o$ $X ⁢ 3 = S ⁢ i , B , C .$

## Revendications

1. Procédé de fabrication d'une aube de turbine par coulée par centrifugation, l'aube de turbine ayant une partie de bord d'attaque présentant une première épaisseur et une partie de bord de fuite présentant une seconde épaisseur inférieure à la première épaisseur, comprenant les opérations suivantes :
a) mise à disposition d'un dispositif de coulée par centrifugation ayant un rotor (1) pouvant tourner autour d'un axe (A), et au moins un creuset (8) logé dans le rotor (1), le creuset ayant au moins une ouverture de sortie,
b) mise à disposition d'un moule (4) ayant une empreinte allongée (20) pour former l'aube de turbine,
c) disposition du moule (4) sur une position radialement vers l'extérieur par rapport au creuset (8) de façon telle qu'une ouverture d'entrée (5) du moule (4) est disposée face à une ouverture de sortie (9) du creuset (8) et, en outre, disposition du moule (4) de façon telle qu'un bord d'attaque du moule (21), qui correspond au bord d'attaque de l'aube de turbine, est dirigé dans une direction opposée au sens de rotation du rotor (1),
d) rotation du rotor (1) tout en forçant une matière fondue métallique (15), au moyen de forces centrifuges, à passer du creuset (8) au moule (4),
e) exercice d'une pression sur la matière fondue (15) forcée dans le moule (4) jusqu'à ce que la température de la matière fondue (15) se solidifiant ait atteint une température de refroidissement prédéfinie, et
f) réduction de la pression lorsque la température de la matière fondue (15) se solidifiant est inférieure à ladite température de refroidissement prédéfinie.

2. Procédé selon l'une des revendications précédentes, selon lequel le bord d'attaque du moule (21) est disposé dans un plan radial (HP) sur un premier angle (α1.), de préférence jusqu'à 30°, par rapport à la direction radiale du rotor (1).

3. Procédé selon l'une des revendications précédentes, selon lequel le premier angle (α1) s'ouvre dans une direction opposée au sens (R) de rotation du rotor (1).

4. Procédé selon l'une des revendications précédentes, selon lequel le bord d'attaque du moule (21) est disposé dans un plan axial (P) sur un second angle (α2), de préférence jusqu'à 30°, par rapport à la direction radiale du rotor (1).

5. Procédé selon l'une des revendications précédentes, selon lequel la température de refroidissement prédéfinie est dans une plage comprise entre 1300 °C et 800°C.

6. Procédé selon l'une des revendications précédentes, selon lequel la pression correspond à la force centrifuge agissant sur la matière fondue (15), multipliée par un facteur compris entre 1,0 et 5,0, au moment où le moule est entièrement rempli.

7. Procédé selon l'une des revendications précédentes, selon lequel la pression est exercée sur la matière fondue (15) durant 1 à 6 minutes après que la température de refroidissement prédéfinie a été atteinte.

8. Procédé selon l'une des revendications précédentes, selon lequel la pression exercée sur la matière fondue (15) est une pression constante ou croissante.

9. Procédé selon l'une des revendications précédentes, selon lequel le rotor (1) effectue une rotation à la même vitesse ou à une vitesse croissante durant l'opération mentionnée au point e).

10. Procédé selon l'une des revendications précédentes, selon lequel la température de refroidissement prédéfinie est dans une plage comprise entre 1050 °C et 800°C.

11. Procédé selon l'une des revendications précédentes, selon lequel la pression est exercée sur la matière fondue (15) en faisant tourner le rotor (1).

12. Procédé selon l'une des revendications précédentes, selon lequel durant les opérations mentionnées aux points d) et e) la matière fondue (15) est sous vide ou sous gaz inerte.

13. Procédé selon l'une des revendications précédentes, selon lequel la matière fondue (15) se solidifiant est refroidie à température ambiante après l'opération mentionnée au point e) à une vitesse de refroidissement comprise entre 50°C et 150°C par heure.

14. Procédé selon l'une des revendications précédentes, selon lequel la matière fondue métallique (15) consiste en un alliage de titane.

15. Procédé selon l'une des revendications précédentes, selon lequel l'alliage de titane comprend Ti et Al comme principaux constituants.

16. Procédé selon les revendications précédentes, selon lequel l'alliage de titane est un alliage à base de γ-TiAl de composition suivants:
$T ⁢ {i}_{45 - 52 ⁢ a ⁢ t . %} ⁢ A ⁢ {l}_{45 - 48 ⁢ a ⁢ t . %} ⁢ X ⁢ {1}_{1 - 3 ⁢ a ⁢ t . %} ⁢ X ⁢ {2}_{2 - 4 ⁢ a ⁢ t . %} ⁢ X ⁢ {3}_{1 ⁢ a ⁢ t ⁢ . %} ,$
où $X ⁢ 1 = C ⁢ r , M ⁢ n , V$ $X ⁢ 2 = N ⁢ b , T ⁢ a , W , M ⁢ o$ $X ⁢ 3 = S ⁢ i , B , C .$
